

Jan. 13, 1953

C. CONE ET AL

2,625,495

HIGH TEMPERATURE CLEANING OF FERROUS METAL

Filed June 4, 1948

2 SHEETS—SHEET 1



Inventors  
CARROLL CONE  
JACK HUEBLER

2312  
*Charles A. Lind*  
Attorney

Jan. 13, 1953

C. CONE ET AL

2,625,495

## HIGH TEMPERATURE CLEANING OF FERROUS METAL

Filed June 4, 1948

2 SHEETS—SHEET 2



BY

INVENTORS  
CAR ROLL CONE  
JACK HI EBLER

Charles A. Lind  
ATTORNEY

ATTORNEY

## UNITED STATES PATENT OFFICE

2,625,495

HIGH-TEMPERATURE CLEANING OF  
FERROUS METAL

Carroll Cone and Jack Huebler, near Toledo, Ohio,  
assignor to Surface Combustion Corporation,  
Toledo, Ohio, a corporation of Ohio

Application June 4, 1948, Serial No. 31,034

10 Claims. (Cl. 134—2)

1

The invention relates to a method of cleaning the surface of a ferrous metal by removing carbonaceous matter and iron oxides in preparation for a coating process such as tinning, galvanizing, plating or painting, and particularly to the cleaning of cold reduced steel strip.

In the manufacture of cold reduced steel strip, the ingot is first reduced by hot rolling to a gauge about four to ten times that of the final gauge. The resulting strip is pickled to remove oxide scale formed during the hot rolling operation, washed with water to remove pickling residues and then oiled in preparation for cold rolling.

After cold rolling, the steel strip carries on its surface a residue of oil and other organic matter which must be removed before the strip is ready for coating. In order to remove such organic matter, it has been customary heretofore to wash the strip in a solvent or alkaline detergent solution, with or without electrolysis. However, since the surface of the strip entering the cold rolling mill is rough and deeply etched, impurities such as oxides, pickling residues and organic matter become imbedded in the surface of the metal during cold rolling. Washing the surface of the cold reduced strip, even when accompanied by electrolysis, removes only superficial impurities and does not remove embedded impurities. If the strip after washing is introduced into a bath of a molten coating metal, as in a galvanizing operation, the rise in temperature causes the embedded oxides and organic matter to generate gases, such as carbon dioxide and water vapor, which are trapped in the metal coating, causing porosity and poor adherence. The embedded impurities also interfere with the wetting and alloying of the coating metal with the base metal. A chemically active coating metal such as zinc or aluminum also may react with the embedded iron oxides to form oxides of the coating metal which interfere with the adherence of the coating.

The principal object of the invention is to provide an improved method of cleaning ferrous metal.

More specific objects and advantages are apparent from the description, in which reference is had to the accompanying drawings illustrating various forms of apparatus for use in the practice of the invention.

Figure I of the drawings is a diagrammatic representation of an apparatus for processing cold reduced steel strip in accordance with the present invention.

Figure II is a similar view showing a preferred form of apparatus.

2

Figure III is a horizontal section taken on line III—III of Figure II.

Figure IV is a detail showing a modification of the apparatus illustrated in Figure II.

5 These specific drawings and the specific description that follows disclose and illustrate, but are not intended to limit the scope of the invention.

United States Patent No. 2,288,980, issued to 10 John J. Turin, suggests that a strip of a ferrous metal be passed through a preheating furnace in which it is exposed to an open flame, to burn off oil, and then passed through a muffle furnace in which it is exposed to an atmosphere formed by 15 burning a hydrocarbon fuel with chlorine and air, to convert iron oxides to iron chlorides. If the step of exposing the strip to an open flame to burn off organic matter had been omitted from the process disclosed in this patent, the only 20 known way of carrying out the process would have been to remove the organic matter from the strip by the usual preliminary washing operation.

It has not been known to be possible heretofore to remove carbonaceous matter and iron oxides simultaneously from the surface of a ferrous metal in a single operation. The present invention is based upon the discovery that it is possible to remove carbonaceous matter and iron oxides simultaneously from the surface of a ferrous metal by heating the metal and exposing it to an atmosphere that is oxidizing to carbon and deoxidizing to iron oxides. As used herein the term "deoxidizing iron oxides" is intended to include conversion of iron oxides to chlorides.

The ferrous metal to be cleaned in the practice of the present invention preferably is preheated before it is introduced into the cleaning atmosphere. The heating of the metal can be carried out more economically by using a preheater than by introducing the cold metal directly into the hot cleaning atmosphere.

Moreover, since the reactions may be reversed by a change in temperature, the same atmosphere that deoxidizes iron oxides at the elevated operating temperature may actually oxidize iron at lower temperatures. Thus the introduction of the cold ferrous metal directly into the cleaning atmosphere may slow down the process by causing initial formation of iron oxides which must be deoxidized after the metal has reached the operating temperature. If the conditions are such that the reactions are liable to be reversed by a drop in temperature, it is desirable also to cool 50 the metal outside of the cleaning atmosphere.

The preheating or outside cooling should be done in a non-oxidizing medium in order to avoid the formation of iron oxides. One convenient method of preheating consists in passing a continuous strip of the metal into the cleaning atmosphere through a bath of molten lead or of a molten salt. Cooling also can be carried out by passing a strip of the metal out of the cleaning atmosphere through such a bath, but when so carried out may produce changes in the metal of the type which ordinarily result from quenching, so that other methods which provide more gradual cooling are ordinarily preferred.

The preheating or cooling may be carried out also by passing a strip of the metal through a preheating chamber, for example a muffle furnace, or a cooling chamber, containing a non-oxidizing atmosphere. Although nitrogen may be used as the non-oxidizing atmosphere in the preheating or cooling chamber, it is usually preferable to use an atmosphere consisting of about 90 mol per cent of nitrogen and 10 mol per cent of hydrogen.

During such preheating, oil and other organic matter on the surface of the metal may be carbonized by decomposition into carbon and free hydrogen or water vapor. In any case, the organic or carbonaceous matter is oxidized to gaseous oxidation products upon exposure to the cleaning atmosphere.

The temperature of the cleaning atmosphere (hereinafter referred to as the "operating temperature") used in the practice of the present invention may range from dark red heat (670-850° F.) upward to well above 1300° F., for example, to about 1700° F., depending upon the particular metallurgical heat treatment that may be desired to fit the ferrous metal for a specific use. The preferred operating temperature is in the range from about 1000° F. to about 1500° F., which is the range of temperature to which cold reduced steel strip ordinarily is heated in annealing. When an operating temperature in the latter range is employed in cleaning cold reduced steel strip in the practice of the invention the desired annealing is accomplished simultaneously with cleaning.

In one embodiment of the present method, the cleaning atmosphere deoxidizes the iron oxides on the surface of the metal by converting them to chlorides. In order to accomplish that result, the cleaning atmosphere may contain a chloride-forming gas such as chlorine. The preferred chloride-forming gas is hydrogen chloride. The atmosphere introduced into the cleaning chamber may be an atmosphere containing gases that react to produce a chloride-forming gas. For example, the atmosphere introduced may contain phosgene and water vapor, which react to form hydrogen chloride and carbon dioxide.

One atmosphere that may be introduced into the cleaning chamber in the practice of the invention contains from 15 to 45 mol per cent of hydrogen chloride, from 10 to 12 mol per cent of carbon dioxide, not more than 2 mol per cent of oxygen and not more than 3 mol per cent of water vapor, the remainder of the atmosphere consisting of nitrogen. If desired, the composition of this atmosphere may be rendered less oxidizing by omitting the free oxygen and adding not more than 3 mol per cent of carbon monoxide and not more than 2 mol per cent of hydrogen, with or without a slight reduction in the carbon dioxide content.

When the cleaning atmosphere contains a

chloride-forming gas the metal preferably is kept at a temperature not less than about 1300° F., to prevent the solidification of ferrous chloride and thus facilitate its removal from the surface of the metal. In the cleaning of cold reduced steel strip in accordance with the present invention, there is no substantial oxidation of the iron and the amount of ferrous chloride produced by reaction with a chloride-forming gas in the cleaning atmosphere is relatively slight as compared with the amount of ferrous chloride that would be produced if it were necessary to remove a heavy coating of iron oxide from the metal. Thus in the present method any coating of ferrous chloride left on the surface of the metal is so slight that it suffices to coat the metal with a chloride flux before introducing it into a galvanizing pot. The necessity for coating the metal with a chloride flux may be avoided by passing the metal through a lead bath (without exposure of the metal to air) at a temperature not less than 1300° F. to remove the slight coating of ferrous chloride. In contrast to the slight amount of ferrous chloride produced in the practice of the present method, the process described in the Turin patent involves heavy oxidation of the strip by the action of the open flame used to burn off the organic matter, and the removal of the resultant heavy coating of iron oxides produces a relatively large amount of ferrous chloride. Thus the strip leaving the cleaning atmosphere in the process of the Turin patent has a relatively heavy coating of ferrous chloride which can be removed satisfactorily only by a washing operation.

In a preferred embodiment of the present method in which the formation of a coating of ferrous chloride on the surface of the metal is avoided altogether, a chloride-forming gas is present in the atmosphere introduced into the cleaning chamber in a concentration low enough to form a final concentration of ferrous chloride vapor less than saturation at the operating temperature, i. e., the concentration of chloride-forming gas in the incoming atmosphere is low enough so that after equilibrium at the operating temperature has been reached in the conversion of the chlorine content of the chloride forming gas to ferrous chloride, the atmosphere still is not saturated with ferrous chloride vapor, and all of the ferrous chloride formed volatilizes. Then, in order to prevent the ferrous chloride from recondensing on the surface of the metal, the metal may be removed from the chloride-containing atmosphere to a cooling chamber as hereinbefore described.

In the apparatus illustrated in Figure I, cold reduced steel strip 2 is unwound from a coil on a pay-out reel 3. At this point, the strip, as obtained from the reduction rolls, has a coating of rolling oil and is hard from cold working. A non-oxidizing preheating medium is provided in the form of molten lead contained in a tank 5, which is heated by a furnace 4 in which the tank is positioned. The strip passes downward from an overhead roller 6 to a submerged roller 7 in the lead bath and thence horizontally to a submerged roller 10. As the strip enters the lead bath, any loose dirt adhering to the oil on the strip is wiped off and floats on the surface of the lead. Some of the oil also is wiped off, and the remainder of the oil is carbonized on the strip. The lead bath also heats the strip to the desired annealing temperature and preheats the strip for the cleaning operation.

From the roller 10 the strip passes upward without exposure to air into an upright retort 11 having a lower extension 12 which dips into the molten lead to form a gas-tight seal. The retort, which contains the cleaning atmosphere, is surrounded by a furnace 13 for maintaining the retort at the desired operating temperature. By the time when the strip reaches an overhead roller 14 at the top of the retort, the cleaning operation has been completed and the strip is ready for cooling. An atmosphere of the composition hereinbefore described, consisting principally of hydrogen chloride, carbon dioxide, and nitrogen, is admitted at the top of the retort through a supply pipe 18 and flows downward through the retort in contact with the upcoming strip. The cleaning atmosphere leaves the lower end of the retort through a waste gas pipe 33.

From the top of the retort, the strip passes into a closed cooling chamber comprising a relatively hot initial portion 16 and a relatively cool final portion 17. The cooling chamber contains rollers 20 to 24 for guiding the strip in its passage through the chamber. In order to prevent oxidation of the strip in the cooling chamber a suitable protective atmosphere is maintained in the chamber. In the apparatus illustrated in Figure I such a protective atmosphere is maintained by permitting some of the atmosphere from the supply pipe 18 to flow into the cooling chamber and out through a vent 32 in the cool portion 17 of the chamber.

Strip cleaned in this apparatus, before it has cooled below galvanizing temperature, may be passed directly from the cooling chamber into a galvanizing pot 15 without any intermediate treatment other than passage through a layer of molten flux contained in a flux box 19. Rollers 25 to 28 conduct the strip through and from the galvanizing pot. From the pot the strip passes through a cooling zone 29 to an overhead roller 30 and thence to a wind-up reel 31.

When the strip to be cleaned is passed through an elongated cleaning chamber and the cleaning atmosphere flows countercurrent to the travel of the strip, the composition and temperature of the atmosphere at the point where the atmosphere leaves and the strip enters the chamber is of no consequence provided that the strip subsequently remains for a sufficient length of time in a portion of the cleaning chamber in which the atmosphere is of a composition and temperature herein specified. Preferably, however, the cleaning atmosphere throughout the entire cleaning chamber has its temperature and composition within the ranges specified herein so that the speed with which the strip travels through the cleaning chamber may be the maximum speed that allows time for oxidation of the carbonaceous matter and deoxidation of the iron oxides.

Figure II illustrates apparatus in which cold reduced steel strip 34 is unwound from a coil on a pay-out reel 35. A preheating zone is provided in the form of an upright tunnel 39, which is heated by a furnace 38 in which the tunnel is positioned, and which contains a non-oxidizing atmosphere. The strip passes beneath a roller 36 and upward over an overhead roller 40. As the strip enters the tunnel through a slot 37 it is heated to an elevated temperature in an atmosphere that is non-oxidizing and may be slightly reducing; nitrogen may be used as the atmosphere, but a mixture of 90 mol per cent nitrogen and 10 mol per cent hydrogen is usually

preferred. Such an atmosphere is admitted at the top of the tunnel through a supply pipe 45 and flows downward through the tunnel in contact with the upcoming strip. This atmosphere leaves the lower end of the tunnel through a waste gas pipe 46.

From the top of the tunnel, the strip passes through a slot 42, over a roller 41 and downward into upright retort 49 having a lower extension 50 which dips into a molten lead bath contained in a tank 51, which is heated by a furnace 16 in which the tank is positioned. The retort 49, which contains the cleaning atmosphere, is maintained at the desired operating temperature by the furnace 38. When the strip reaches the lead bath below the retort, the gaseous cleaning operation has been completed and the strip is clean except for a coating of ferrous chloride which is removed in the lead bath. The cleaning atmosphere is admitted at the bottom of the retort through a supply pipe 48 and flows upward through the retort in contact with the downward moving strip. The atmosphere leaves the upper end of the retort through a waste gas pipe 47.

25 The strip is conducted through the lead bath by rollers 53 and 54. The ferrous chloride in the lower extension 50 of the retort 49 is kept from attaining an unduly high level by an overflow 75.

From the lead bath, the strip passes into a closed cooling chamber comprising a relatively hot initial portion 55 and a relatively cool final portion 56. The intermediate portion of the cooling chamber contains rollers 57 to 60 for guiding the strip in its passage through the chamber. In order to prevent oxidation of the strip in the cooling chamber a suitable protective atmosphere is maintained in the chamber. In the apparatus illustrated in Figure II such a protective atmosphere is admitted at the cool end of the cooling chamber through a supply pipe 62 and flows through the cooling chamber and out through a waste gas pipe 61.

Strip cleaned in this apparatus, before it has cooled below galvanizing temperature, may be passed directly from the cooling chamber into a galvanizing pot 68 without any intermediate treatment. Rollers 63 to 67 conduct the strip to, through and from the galvanizing pot. From the pot the strip passes to an overhead roller 69 and thence to a wind-up reel 70.

Figure III shows a section through the furnace 38. The strip 34 is represented in section inside the tunnel 39 and retort 49.

Figure IV illustrates an alternative connection between the cleaning zone 49 and the cooling zone 55 which connection eliminates the lead bath contained in the tank 51. This alternative connection can be used when the atmosphere in the cleaning zone is such that carbonaceous matter is oxidized and iron oxides are deoxidized simultaneously without the formation of a coating of ferrous chloride, as described herein. When this alternative connection is used, the strip 34 passes downward from the retort 49, through a slot 77, beneath rollers 72 and 73, and upward into the cooling zone 55. In the modification illustrated in Figure IV the protective atmosphere of the cooling zone is exhausted through a waste gas pipe 74. When the cleaning atmosphere that is used is oxidizing to carbonaceous matter because of the presence of  $\text{CO}_2$  or  $\text{H}_2\text{O}$  and is simultaneously reducing to iron oxides because of the presence of  $\text{CO}$ ,  $\text{H}_2$  or  $\text{HCl}$ , this is true because the composition of the cleaning atmosphere has been regulated so that cer-

tain equilibrium conditions are exceeded (causing a tendency for the oxidation of carbon) at the same time that certain other equilibrium conditions are exceeded (causing a tendency for the reduction of iron oxides). When it is desired to oxidize carbon (at atmospheric pressure) by the action of water vapor, the initial concentration of  $H_2O$  should exceed (0.01) (as used herein, a gas concentration expressed as a figure in parentheses refers to the partial pressure of that gas in atmosphere), and the concentration should at all times be such that

$$(1) \quad \log_{10} \frac{(CO)(H_2)}{(H_2O)} > 7.543 - \frac{12,750}{t+460}$$

in which  $(CO)$ ,  $(H_2)$  and  $(H_2O)$  are the gas concentrations of carbon monoxide, hydrogen and water vapor, respectively, and  $t$  is the operating temperature in degrees F. When it is desired to oxidize carbon by the action of carbon dioxide, the initial concentration of  $CO_2$  should exceed (0.05), and the concentration should at all times be such that

$$(2) \quad \log_{10} \frac{(CO_2)}{(CO)^2} > \frac{16,000}{t+460} - 9.19$$

in which  $(CO_2)$  and  $(CO)$  are the gas concentrations of carbon dioxide and carbon monoxide, respectively, and  $t$  is the operating temperature in degrees F. When it is desired to deoxidize iron oxides by the action of hydrogen, the initial concentration of  $H_2$  should exceed (0.05), and the concentration should at all times be such that

$$(3) \quad \log_{10} \frac{(H_2)}{(H_2O)} > \frac{1487}{t+460} - 0.450$$

in which  $(H_2)$  and  $(H_2O)$  are the gas concentrations of hydrogen and water vapor, respectively, and  $t$  is the operating temperature in degrees F. When it is desired to deoxidize iron oxides by the action of carbon monoxide, the initial concentration of  $CO$  should exceed (0.05), and the concentration should at all times be such that

$$(4) \quad \log_{10} \frac{(CO)}{(CO_2)} > 1.200 - \frac{1800}{t+460}$$

in which  $(CO)$  and  $(CO_2)$  are the gas concentrations of carbon monoxide and carbon dioxide, respectively, and  $t$  is the operating temperature in degrees F. When it is desired to deoxidize iron oxides by the action of hydrogen chloride, the initial concentration of  $HCl$  should exceed (0.01), and the concentration should at all times be such that

$$(5) \quad \log_{10} \frac{(H_2)}{(HCl)^2} < \frac{9770}{t+460} - 4.44$$

in which  $(H_2)$  and  $(HCl)$  are the gas concentrations of hydrogen and hydrogen chloride, respectively, and  $t$  is the operating temperature in degrees F.

As explained hereinbefore, it is sometimes possible to clean steel in the practice of the invention under such conditions that the cleaning atmosphere exhausted from the cleaning zone is not within the limits defined by Inequalities 1 to 5. When this is true, the equipment is being operated inefficiently, and more strip could be cleaned by keeping the entire cleaning atmosphere within the prescribed limits and moving the strip through the cleaning zone at a greater speed. Consequently, in order that the equipment may be operated efficiently, it is preferred that the gas exhausted from the cleaning zone be within the prescribed limits.

In the analysis of gas compositions that are used in the practice of the invention it is necessary that certain precautions be taken to ensure accurate results. It is understood that a mixture of  $CO$ ,  $CO_2$ ,  $H_2$ ,  $H_2O$  and  $HCl$  is capable of any of a number of equilibria. What the equilibrium is for any mixture that contains these materials is a function of temperature, so that a gas composition that is not within the limits prescribed for use in the practice of the invention could, if analyzed at a different temperature under equilibrium conditions, appear to be one within the limits. Conversely, a gas composition within the prescribed limits could, if analyzed at a different temperature under equilibrium conditions, appear not to be within the limits. Thus it is important that the gas analysis be made in such a way as to avoid these possible sources of error. It has been found that changes in the composition of the mixture of gases used as the cleaning atmosphere occur at an extremely slow rate at room temperature. Therefore, the expedient of rapidly cooling a sample of the atmosphere ensures sufficiently accurate results; rapid cooling to room temperature has the effect of "freezing" the gas composition. Any  $HCl$  in the atmosphere should be removed before the rapid cooling to prevent it from dissolving in condensed water vapor to form a hydrochloric acid solution which then absorbs  $CO_2$  so as to make analysis more difficult.

The atmosphere that is maintained in the cooling zone should not be oxidizing to the cleaned steel surface, and best results are frequently obtained when this atmosphere is slightly reducing. Thus, it is possible to conduct the cleaning operation with a nitrogen atmosphere in the cooling zone, but it is usually preferable that the atmosphere be slightly reducing, a mixture of 90 mol per cent nitrogen and 10 mol per cent hydrogen being a desirable reducing atmosphere.

Because the cleaning atmosphere that is used in the practice of the invention may be effective at a given operating temperature, but either oxidizing to steel or reducing to carbon at a slightly lower temperature, it is usually desirable to avoid any leakage of the cleaning atmosphere into either the preheating zone or the cooling zone. This can be accomplished readily by operating the cooling and preheating zones at a pressure slightly greater than the pressure of the cleaning zone, so that any flow of gas from one zone to another will be toward the cleaning zone. Except for the slightly higher pressures in the cooling and preheating zones, it is usually desirable to conduct the cleaning operation at or about atmospheric pressure.

Ferrous metal can be cleaned, in the practice of the invention, without pretreatment, carbonaceous matter and iron oxides being removed chemically as described herein. However, particularly when the metal to be cleaned has a heavy covering of carbonaceous matter which is loosely adherent to the surface of the metal, it may be advantageous to subject the metal to a pretreatment in the form of a washing operation to remove surface carbonaceous matter so that there is less to be removed by the method of the invention, which is particularly efficient in that it removes carbonaceous matter that the washing operation does not reach, and simultaneously reduces iron oxides.

In general, the minimum time that the ferrous metal should remain in contact with the cleaning atmosphere depends upon the operating

temperature and upon the amount of carbonaceous material and iron oxides to be removed from the metal. Thus, using an operating temperature of about 1000° F. it is practical to conduct ferrous metal that has been washed to remove some surface carbonaceous matter through the cleaning atmosphere at such a rate that it is subjected to cleaning conditions for a time as short as about 30 seconds, although it is usually preferable to allow about an extra five seconds to make certain that the metal will be thoroughly cleaned. When the operating temperature is about 1500° F. such metal can be conducted through the cleaning atmosphere at such a rate that it is subjected to cleaning conditions for a time as short as about five seconds, although it is usually preferable to allow about an extra two seconds to make certain that the metal will be thoroughly cleaned. When the metal to be cleaned has a heavy surface coating of carbonaceous matter it may be desirable to maintain the metal in contact with the cleaning atmosphere for about twice the time indicated for metal that has been washed. When intermediate operating temperatures are used, the minimum time that the metal should be in contact with the cleaning atmosphere is intermediate between the times indicated. There is no theoretical reason why the metal cannot be left in contact with the cleaning atmosphere for comparatively long periods of time, provided that the composition of the atmosphere is within the limits described. However, in practice it is usually desirable to operate the cleaning equipment at such a rate that the maximum amount of metal is cleaned during the operation. Therefore, it is ordinarily preferable that the metal be conducted through the cleaning atmosphere at about the maximum rate that gives efficient cleaning.

A preferred embodiment of the invention involves the use of a cleaning atmosphere which comprises hydrogen and water vapor. An example of such an atmosphere is one containing 20 mol per cent of hydrogen, 5 mol per cent of water vapor, and 75 mol per cent of nitrogen. Such an atmosphere can be used within the preferred range of operating temperatures, i. e., at temperatures between about 1000° F. and about 1500° F.

The way in which Inequalities 1 through 5 can be used to determine operating conditions which will be simultaneously oxidizing to carbonaceous matter and reducing to iron oxides is illustrated by the following calculations:

Consider an operating temperature of 1200° F. and an atmosphere that contains only carbon monoxide, carbon dioxide, and a diluent, such as nitrogen.

From Inequality 4,

$$\log_{10} \frac{(\text{CO})}{(\text{CO}_2)} > 1.200 - \frac{1200}{1660}$$

From Inequality 2,

$$\log_{10} \frac{(\text{CO}_2)}{(\text{CO})^2} > \frac{16000}{1660} - 9.19$$

From the ratios,

$$\log_{10} \frac{(\text{CO})}{(\text{CO}_2)} > 0.074$$

and

$$\log_{10} \frac{(\text{CO}_2)}{(\text{CO})^2} > 0.35$$

can be calculated a series of gas compositions of carbon monoxide, carbon dioxide and an in-

ert gas, such as nitrogen, which will be simultaneously oxidizing to carbonaceous matter and reducing to iron oxides. For example,

Assume that the concentration of carbon monoxide is (0.07); then,

$$(6) \quad \log_{10} \frac{(\text{CO})}{(\text{CO}_2)} = \log_{10} \frac{0.07}{(\text{CO}_2)} > 0.074$$

and

$$(7) \quad \log_{10} \frac{(\text{CO}_2)}{(\text{CO})^2} = \log_{10} \frac{(\text{CO}_2)}{(0.07)^2} > 0.35$$

Therefore, from (6),  $(\text{CO}_2)$  must be less than the value that makes

$$\log_{10} \frac{0.07}{(\text{CO}_2)} = 0.074$$

and, from (7),  $(\text{CO}_2)$  must be greater than the value that makes

$$\log_{10} \frac{(\text{CO}_2)}{(0.0049)} = 0.35$$

Solution of these two equations gives the limits of concentration within which, at 1200° F., carbon dioxide can be present in a gas composition

25 in which the partial pressure of carbon monoxide is 0.07 atmosphere, that is simultaneously oxidizing to carbonaceous matter and deoxidizing to iron oxides, if in addition to the carbon monoxide and carbon dioxide the composition contains only an inert gas such as nitrogen. By similar calculations, assuming different temperatures and different carbon monoxide concentrations, the limits of other suitable gas compositions that consist of carbon monoxide, carbon dioxide and an inert gas can be calculated.

30 If the gas composition that is selected for use in the cleaning zone is one whose components are capable of reaction, i. e., are out of equilibrium, the equilibrium composition of the gas at the desired operating temperature should be determined in order to ascertain whether or not the equilibrium composition is within the limited defined by Inequalities 1 through 5 so that the gas, at equilibrium, is simultaneously oxidizing to carbonaceous matter and deoxidizing to iron oxides. For example, if the gaseous atmosphere contains  $\text{H}_2$ ,  $\text{H}_2\text{O}$ ,  $\text{CO}$  and  $\text{CO}_2$ , the stable mixture is one represented by the dynamic equilibrium.



35 The equilibrium concentrations of the various components depend upon temperature. It is usually preferable that the cleaning atmosphere be one which, when it reaches equilibrium at the operating temperature, is simultaneously oxidizing to carbonaceous matter and deoxidizing to iron oxides so that there is not the possibility that, during the cleaning reaction, the gas will, in approaching equilibrium, become, for example, oxidizing to iron.

40 A trial and error method may be used for determining the gas compositions that are practical for use in the practice of the invention; instead of the method of calculation indicated in the preceding paragraphs. This is done by supplying to a cleaning zone a gas of a composition that is known, from a consideration of the relationships shown in Inequalities 1 through 5, to be simultaneously oxidizing to carbonaceous matter and deoxidizing to iron oxides, passing the gas through the cleaning zone at the desired operating temperature in contact with the metal to be cleaned and then analyzing the outgoing gas. It is then determined whether or not the analysis indicates that the gas (according to Inequalities

## 11

1 through 5) is simultaneously oxidizing to carbonaceous matter and deoxidizing to iron oxides. This method is usually found to be simpler than theoretical calculations based upon equilibrium considerations and rates of reaction.

As has been stated hereinbefore, a gaseous composition that is oxidizing to carbon and deoxidizing to iron oxides at a given temperature may be oxidizing to both carbon and iron oxides at lower temperatures. For example, the relationships in Inequalities 2 and 4 are such that, when  $t$  is less than about 900° F., there are no compositions of carbon monoxide, carbon dioxide and an inert gas that are simultaneously oxidizing to carbonaceous matter and deoxidizing to iron oxides, because the minimum concentration of  $\text{CO}_2$  that is possible (to give a gas that is oxidizing to carbonaceous material) is higher than the maximum concentration of  $\text{CO}_2$  that is permissible (to give a gas that is not oxidizing to iron). As a consequence, it is usually preferred that the metal to be cleaned be heated, then exposed to the cleaning atmosphere, at a temperature in the operating range, and then cooled in an atmosphere different from the cleaning atmosphere. The cooling atmosphere should be non-oxidizing to the metal, and preferably slightly reducing.

A preferred embodiment of the invention (to which the equipment generally illustrated in Figure II is well adapted) involves the use of a cleaning atmosphere that contains HCl in such an amount that it converts iron oxides to ferrous chloride, but does not produce an amount of ferrous chloride sufficient to saturate the cleaning atmosphere with ferrous chloride vapor at the operating temperature. In practicing this embodiment of the invention, the modification illustrated in Figure IV is used, because the ferrous chloride formed by reaction of the HCl with iron oxides is vaporized and carried from the equipment with the cleaning atmosphere, so that little or no ferrous chloride remains on the cleaned metal and use of a lead bath is unnecessary.

The instant invention is of particular value because it provides a method for cleaning a ferrous metal that is at the same time efficient, capable of application to simple equipment, and inexpensive (as compared with known ways of cleaning ferrous metals).

Molten metal or salt baths can be used in place of inert gas atmospheres as either preheating or cooling media.

## Example 1

A gas composition comprising carbon monoxide, 55 carbon dioxide, hydrogen, water vapor and nitrogen can be prepared by burning methane in air according to the following procedure:

Methane is burned in air (using a 1:6 volume ratio of methane to air), and the products of 60 combustion are partially dehydrated by cooling them to 45° F. The resulting gas composition, which contains (per 100 mols of gas) 10.2 mols of CO, 5.2 mols of  $\text{CO}_2$ , 12.5 mols of  $\text{H}_2$ , 1.0 mol of  $\text{H}_2\text{O}$  and 71.1 mols of  $\text{N}_2$ , is reacted to equilibrium at 1250° F. (about 30 minutes). At equilibrium the gas contains (per 100 mols of gas) 11.4 mols of CO, 4.0 mols of  $\text{CO}_2$ , 11.3 mols of  $\text{H}_2$ , 2.2 mols of  $\text{H}_2\text{O}$  and 71.1 mols of  $\text{N}_2$ . This mixture (the equilibrium mixture of 1250° F.) is simultaneously 65 oxidizing to carbonaceous matter and deoxidizing to iron oxides, and can be used to clean ferrous metals by simultaneously oxidizing carbonaceous matter and deoxidizing iron oxides, care being taken to use a sufficient quantity of the gas so 70

## 12

that all the carbonaceous matter and iron oxides are removed from the metal.

## Example 2

5 A ferrous metal is cleaned by an atmosphere that is simultaneously oxidizing to carbonaceous matter and reducing to iron oxides, prepared as follows:

The cleaning atmosphere is prepared by burning a gaseous mixture of methane (1 part by volume), chlorine (2 parts by volume) and air (3.8 parts by volume), and combining 15 parts by volume of this gas with 85 parts by volume of another gas prepared by burning methane (1 part by volume) with air (6.67 parts by volume) and partially dehydrating the combustion products by cooling them to 40° F.; the resulting cleaning atmosphere contains (per 100 mols of the atmosphere) 6.3 mols of CO, 7.5 mols of  $\text{CO}_2$ , 8.3 mols of  $\text{H}_2$ , 0.7 mol of  $\text{H}_2\text{O}$ , 70.3 mols of  $\text{N}_2$  and 6.9 mols of HCl.

If this cleaning atmosphere is reacted with iron oxides at 1250° F. until equilibrium is reached, the final composition of the gas would consist of (per 100 mols of original gas) 8.3 mols of CO, 5.5 mols of  $\text{CO}_2$ , 7.0 mols of  $\text{H}_2$ , 2.8 mols of  $\text{H}_2\text{O}$ , 70.3 mols of  $\text{N}_2$ , 5.3 mols of HCl and 0.8 mol of  $\text{FeCl}_2$ . By means of Inequalities 1 through 5 it can be shown that this final composition is oxidizing to carbonaceous matter but not oxidizing to iron. The concentration of  $\text{FeCl}_2$  in this final composition is not sufficient to saturate the atmosphere with that component at the operating temperature. Therefore, this cleaning atmosphere can be used at an operating temperature of 1250° F., and, even if the reaction with iron oxides goes to equilibrium, the final gas is still not oxidizing to iron and is still not saturated with ferrous chloride. Of course, less reaction with iron oxides results in a gas within the indicated ranges of composition. In the use of this cleaning atmosphere in the apparatus illustrated in Figure I or Figure II, the rate of flow of the cleaning atmosphere should be just great enough to remove all the iron oxide from the metal at 1250° F. Such a rate of flow is ordinarily enough also to remove all carbonaceous matter from the metal.

## Example 3

A ferrous metal is cleaned by an atmosphere that is simultaneously oxidizing to carbonaceous matter and reducing to iron oxides, prepared as follows:

The cleaning atmosphere is prepared by burning a gaseous mixture of anhydrous ammonia and chlorine and diluting with partially dehydrated products of the complete combustion of ammonia with air to produce a gaseous mixture containing (per 100 mols of the cleaning atmosphere) 0.3 mol of  $\text{H}_2\text{O}$ , 95.7 mols of  $\text{N}_2$  and 4.0 mols of HCl.

If this cleaning atmosphere is reacted with iron oxides at 1250° F. until equilibrium is reached, the final composition of the gas would consist of (per 100 mols of original gas) 0.9 mol of  $\text{H}_2$ , 0.3 mol of  $\text{H}_2\text{O}$ , 95.7 mols of  $\text{N}_2$ , 2.2 mols of HCl and 0.9 mol of  $\text{FeCl}_2$ . The concentration of  $\text{FeCl}_2$  in this final composition is not sufficient to saturate the atmosphere with that component at the operating temperature. Therefore, this cleaning atmosphere can be used at an operating temperature of 1250° F., and, even if the reaction with iron oxides goes to equilibrium, the final gas is still not oxidizing to iron and is still not saturated with ferrous chloride.

## Example 4

A ferrous metal is cleaned by an atmosphere that is simultaneously oxidizing to carbonaceous matter and reducing to iron oxides, prepared as follows:

The cleaning atmosphere is prepared by burning anhydrous ammonia with chlorine and diluting with partially dehydrated products of the incomplete combustion of ammonia with air to produce a gaseous mixture containing (per 100 mols of the cleaning atmosphere) 5.0 mols of H<sub>2</sub>, 1.0 mol of H<sub>2</sub>O, 87.0 mols of N<sub>2</sub>, and 7.0 mols of HCl. If this cleaning atmosphere is reacted with iron oxides at 1250° F. until equilibrium is reached, the final composition of the gas would consist of (per 100 mols of original gas) 5.9 mols of H<sub>2</sub>, 1.0 mol of H<sub>2</sub>O, 87.0 mols of N<sub>2</sub>, 5.2 mols of HCl and 0.9 mol of FeCl<sub>2</sub>. The concentration of FeCl<sub>2</sub> in this final composition is not sufficient to saturate the atmosphere with that component at the operating temperature. Therefore, this cleaning atmosphere can be used at an operating temperature of 1250° F., and, even if the reaction with iron oxides goes to equilibrium, the final gas is still not oxidizing to iron and is still not saturated with ferrous chloride.

This is a continuation-in-part of application Serial No. 595,208, filed May 22, 1945, and now abandoned.

Having described the invention, we claim:

1. A method of cleaning ferrous metal whose surface carries carbonaceous matter and iron oxides that comprises the step of exposing said metal at a temperature of 670° F.-1700° F. to an atmosphere that contains both (1) a gas that is oxidizing to carbon and (2) a second gas that is deoxidizing to iron oxides, and so adjusting the length of time of such exposure and the concentrations of gas (1) and of gas (2) in the atmosphere during such exposure that substantially complete removal of both the carbonaceous matter and the iron oxides is accomplished simultaneously.

2. A method of cleaning ferrous metal whose surface carries carbonaceous matter and iron oxides that comprises the step of exposing said metal at a temperature of 670° F.-1700° F. to an atmosphere that contains both (1) an oxidizing gas from the class consisting of H<sub>2</sub>O, CO<sub>2</sub> and mixtures thereof and (2) a deoxidizing gas from the class consisting of H<sub>2</sub>, Cl<sub>2</sub>, CO, HCl and mixtures thereof, and so adjusting the length of time of such exposure and the concentrations of gas (1) and of gas (2) in the atmosphere during such exposure that substantially complete removal of both the carbonaceous matter and the iron oxides is accomplished simultaneously.

3. A method as claimed in claim 1 wherein the temperature is 1000° F.-1500° F.

4. A method as claimed in claim 2 wherein the temperature is 1000° F.-1500° F.

5. A method as claimed in claim 4 wherein said atmosphere is obtained by subjecting to the operating conditions described a gaseous mixture consisting of 15-45 mol per cent HCl, 10-12 mol per cent CO<sub>2</sub>, not more than 2 mol per cent O<sub>2</sub>, not more than 3 mol per cent H<sub>2</sub>O and the remainder N<sub>2</sub>.

6. A method of cleaning ferrous metal whose surface carries carbonaceous matter and iron oxides that comprises the steps of exposing said metal at a temperature of 670° F.-1700° F. to an atmosphere that contains both (1) a gas that is oxidizing to carbon and (2) a second gas that is deoxidizing to iron oxides, and so adjusting the length of time of such exposure and the concentrations of gas (1) and of gas (2) in the atmosphere during such exposure that substantially complete removal of both the carbonaceous matter and the iron oxides is accomplished simultaneously, and then cooling said metal in an atmosphere that is inert to said metal.

7. A method of cleaning ferrous metal whose surface carries carbonaceous matter and iron oxides that comprises the steps of preheating said metal in a non-oxidizing medium and then exposing said metal at a temperature of 670° F.-1700° F. to an atmosphere that contains both (1) a gas that is oxidizing to carbon and (2) a second gas that is deoxidizing to iron oxides, and so adjusting the length of time of such exposure and the concentrations of gas (1) and of gas (2) in the atmosphere during such exposure that substantially complete removal of both the carbonaceous matter and the iron oxides is accomplished simultaneously.

8. A method of cleaning ferrous metal whose surface carries carbonaceous matter and iron oxides that comprises the steps of exposing said metal at a temperature of 670° F.-1700° F. to an atmosphere that contains both (1) an oxidizing gas from the class consisting of H<sub>2</sub>O, CO<sub>2</sub> and mixtures thereof and (2) a deoxidizing gas from the class consisting of H<sub>2</sub>, Cl<sub>2</sub>, CO, HCl and mixtures thereof, and so adjusting the length of time of such exposure and the concentrations of gas (1) and of gas (2) in the atmosphere during such exposure that substantially complete removal of both the carbonaceous matter and the iron oxides is accomplished simultaneously, and then cooling said metal in a different atmosphere that is inert to said metal.

9. A method as claimed in claim 8 wherein the second atmosphere is at a higher pressure than the first atmosphere.

10. A method as claimed in claim 8 in which the initial composition of the first atmosphere includes hydrogen chloride in a concentration low enough to form a final concentration of ferrous chloride vapor less than saturation at the operating temperature.

CARROLL CONE.  
JACK HUEBLER.

## REFERENCES CITED

The following references are of record in the file of this patent:

## UNITED STATES PATENTS

| Number    | Name       | Date          |
|-----------|------------|---------------|
| 2,199,418 | Redmond    | May 7, 1940   |
| 2,288,980 | Turin      | July 7, 1942  |
| 2,347,527 | Vanderbilt | Apr. 25, 1944 |
| 2,437,528 | Hodil      | Mar. 9, 1948  |